

## UNITED STATES PATENT OFFICE

2,163,934

## COPY SHEET

Howard E. Collins, La Grange, Ill., assignor to  
 Ditto, Incorporated, Chicago, Ill., a corpora-  
 tion of West Virginia

No Drawing. Application March 5, 1938,  
 Serial No. 194,112

11 Claims. (Cl. 41—31.6)

This invention relates to an improvement in copy sheets and more particularly to master copy sheets, adapted to give designs of higher color intensity in a duplicating process wherein a design to be reproduced is applied to a master copy sheet by typewriting and the like, the design on the master copy sheet contacted with a duplicating mass, and copies made by contacting copy sheets in succession with the design on the duplicating mass.

In the usual hectograph duplicating process a design formed of a water and glycerin soluble dye is applied to an ordinary paper sheet such as bond paper to form a master copy. The design on the master copy is then contacted with a duplicating mass consisting of gelatin, glycerin and water, whereupon the dye of the design is largely transferred to the hectograph mass, forming a reverse image of the design. Copies are then made by contacting copy sheets with the design on the hectograph mass. Where the dye used in forming the designs is not readily soluble in water and glycerin, the color of the design on the copies is of poor intensity after only a few copies have been made. This is particularly true of black basic nigrosine, and also of highly light absorbent combinations of basic dyes such as the mixtures of fuchine and malachite green in the proportion of 1:2.

In accordance with this invention there is distributed on the surface of a copy sheet a glycerin miscible solvent which has a greater solvent power than glycerin for basic nigrosine and other like transfer dyes.

One embodiment of the invention is a paper copy sheet having a coating of a relatively non-volatile solvent selected from the group consisting of homologs of "Cellosolve" (ethylene glycol ethyl ether) and "Carbitol" (di-ethylene glycol ethyl ether).

The solvent may be applied to the paper sheet and bound thereto by any suitable means known to the art. It may be incorporated with the paper pulp during the process of manufacture of the paper so that the finished paper contains the solvent uniformly distributed in it. It may also be applied to a paper sheet coated with some suitable substance which will absorb the solvent or the solvent may be applied directly to the surface of the sheet either alone or in a mixture with other constituents.

The following examples are given to illustrate the invention:

## Example 1

A sheet of sulphite bond paper 17" x 22" is coated with the following composition:

|                                                                 |       |    |   |
|-----------------------------------------------------------------|-------|----|---|
| Dimethoxytetra glycol (dimethyl ether of tetra ethylene glycol) | cc    | 10 | 5 |
| Water                                                           | cc    | 30 |   |
| Starch                                                          | grams | 3  |   |

The amount of coating is 0.8 gram per 17" x 22" sheet of paper.

A design was produced on this coated copy sheet by typing, using a black carbon paper containing a basic nigrosine dye. This sheet containing the black dye design was then applied to a hectograph blanket of the ordinary type consisting, for example, of glue or gelatin, 30 parts by weight, water, 35 parts and glycerin 300 parts, whereupon the black dye of the design was largely transferred to the hectograph mass. Copies were then produced from the hectograph mass in the conventional manner without application of any solvent or resort to any special procedure. It was found that at least thirty-five intense black copies could be produced in this manner.

## Example 2

A sheet of paper was coated with the following composition:

|                                                 |       |    |    |
|-------------------------------------------------|-------|----|----|
| Butyl carbitol (di-ethylene glycol butyl ether) | cc    | 10 | 30 |
| Water                                           | cc    | 30 |    |
| Gelatin                                         | grams | 3  |    |
| Kaolin                                          | do    | 10 |    |

A design was produced on this sheet by typing, using a carbon paper containing a mixture of fuchsin and malachite green in proportions of 1:2. The sheet containing the design was then used to obtain copies by the ordinary hectograph process. Similar results as for Example 1 were obtained.

While there has been shown and described certain embodiments of the invention, it is to be understood that it is capable of many modifications. Changes in the proportions, and substitution of equivalent materials may be made without departing from the spirit and scope of the invention as described in the appended claims, in which it is the intention to claim all novelty inherent in the invention as broadly as possible in view of the prior art.

I claim:

1. The process of reproducing designs which comprises applying a design formed of a soluble dye to a sheet having uniformly distributed on

- its surface a glycerin miscible solvent having a greater solvent power than glycerin for said dye, and contacting the design on said sheet with a hectograph copy mass to transfer the design to 5 said mass.
2. The process of reproducing designs which comprises applying a design formed of a basic nigrosine dye to the surface of a sheet containing on its surface a glycerin miscible solvent having a greater solvent power than glycerin for 10 said basic nigrosine dye, contacting the design on said sheet with a copy pad to transfer the design to said pad, and contacting a copy sheet with the copy pad to transfer the design to said 15 copy sheet.
3. A copy sheet having distributed on its surface a composition comprising a dye solvent and an absorbent substance adapted to retain the dye solvent at the surface of the sheet, said dye 20 solvent being of sufficiently low volatility as to remain in the sheet over a prolonged period of time under normal conditions, of greater solvent power than glycerin, and soluble in glycerin and water.
- 25 4. A copy sheet having distributed on its surface a composition comprising a solvent selected from the group consisting of ethers of glycols and polyglycols, admixed with an absorbent substance adapted to retain the solvent at the 30 surface of the sheet.
5. A copy sheet having distributed on its surface a composition comprising di-ethylene glycol butyl ether and an absorbent substance adapted to retain the di-ethylene glycol butyl ether at 35 the surface of the sheet.
6. A copy sheet having distributed on its surface a composition comprising di-methoxytetra glycol and an absorbent substance adapted to re-
- tain the di-methoxytetra glycol at the surface of the sheet.
7. A copy sheet having distributed on its surface a composition comprising di-ethylene glycol butyl ether, gelatin, and an absorbent clay. 5
8. A copy sheet having distributed on its surface a composition comprising di-methoxytetra glycol and starch.
9. The process of reproducing designs which comprises applying a design formed of a water 10 or alcohol soluble dye to a sheet having uniformly distributed on its surface a composition comprising a solvent from the group consisting of ethers of glycols and polyglycols, contacting the design on said sheet with a copy pad to transfer 15 the design to said pad, and contacting a copy sheet with the copy pad to transfer the design to said copy sheet.
10. The process of reproducing designs which comprises applying a design formed of a water 20 or alcohol soluble dye to a sheet having uniformly distributed on its surface a composition comprising di-ethylene glycol butyl ether, contacting the design on said sheet with a copy pad to transfer 25 the design to said pad, and contacting a copy sheet with the copy pad to transfer the design to said copy sheet.
11. The process of reproducing designs which comprises applying a design formed of a water 30 or alcohol soluble dye to a sheet having uniformly distributed on its surface a composition comprising di-methoxytetra glycol, contacting the design on said sheet with a copy pad to transfer the design to said pad, and contacting a copy sheet with the copy pad to transfer the design 35 to said copy sheet.

HOWARD E. COLLINS.